

## UNITED STATES PATENT OFFICE.

CHARLES H. KECK, OF NEW YORK, N. Y.

## PROPELLANT POWDER.

No Drawing.

Application filed July 27, 1926. Serial No. 125,284.

(GRANTED UNDER THE ACT OF MARCH 3, 1883; 22 STAT. L. 625.)

The subject of this invention is a propellant powder.

Attempts have been made to provide a flashless gun powder by the introduction of various ingredients designed to produce cooling of the gases of combustion prior to emission from the muzzle or designed to produce gases whose temperature as discharged from the muzzle is below that required for further combustion of the gases.

These attempts have not resulted in the production of a consistently uniform flashless powder which will effectively suppress the flash under varying conditions of use and increasing the proportion of flash reducing agent results in the production of smoke.

The principal object of the present invention is to utilize an ingredient which will unvaryingly produce the desired flashless result, reduce the hygroscopicity of the powder and also serve as a stabilizer.

In accomplishing this purpose I propose to incorporate in a nitrocellulose powder nitrated linseed oil or nitrated castor oil. As an example of powders of this type several which proved very successful consist of the following composition.

|                           | Per cent. |
|---------------------------|-----------|
| Nitrocellulose (11—13.5N) | 97        |
| Nitrated linseed oil      | 3         |
| Nitrocellulose (11—13.5N) | 97        |
| Nitrated castor oil       | 3         |

These proportions may be varied and the oil may be reduced to 1% or increased to 15% to give reduction in flash without producing smoke. With an oil content of 5 to 10% nitrocellulose powder is brought within the hygroscopicity limits for an improved powder.

In addition to giving good uniformity,

velocity and pressure incorporation of the oils increase the shrinkage of the colloid giving a denser powder and therefore increasing the capacity of the cartridge case.

These oils are better stabilizers for nitrocellulose powder than diphenylamine which is universally used for this purpose, the results of the various tests indicating a higher order of stability.

Vegetable oils, such as linseed oil and castor oil may be nitrated as follows:

## (a) Acid.

|                | Per cent. |
|----------------|-----------|
| Nitric acid    | 19 55     |
| Sulphuric acid | 68        |
| Water          | 13        |

Nitric ratio 0.3 pounds  $HNO_3$  to one pound of castor oil or linseed oil.

## (b) Nitration.

Castor oil, mixed with equal parts (by weight) of glacial acetic acid. Linseed oil mixed with  $\frac{1}{2}$  its weight of glacial acetic acid.

The mixtures are nitrated with the above nixed acid at a temperature below  $15^\circ C$ . After all the acid has been added, the mixture is cooked for  $\frac{1}{2}$  hour at the same temperature.

I claim:

1. A powder including nitrocellulose to 99% and nitrated castor oil 1 to 15%.
2. A powder including nitrocellulose to 99% and nitrated vegetable oil 1 to 15%.
3. A nitrocellulose powder in which is incorporated nitrated vegetable oil.
4. A nitrocellulose powder in which is incorporated nitrated castor oil.

CHARLES H. KECK.